

June 18, 1929.

M. L. GORDON

1,717,769

COMPOSITE BITUMINOUS PAVEMENT AND METHOD OF LAYING THE SAME

Filed June 21, 1926



INVENTOR.

*Morris L. Gordon*

BY

*Lounse, Loftus & Abbott*

ATTORNEYS.

Patented June 18, 1929.

1,717,769

# UNITED STATES PATENT OFFICE.

MORRIS L. GORDON, OF BURLINGAME, CALIFORNIA.

## COMPOSITE BITUMINOUS PAVEMENT AND METHOD OF LAYING THE SAME.

Application filed June 21, 1926. Serial No. 117,409.

This invention relates to a composite bituminous pavement and the method of laying the same.

Practically all bituminous pavements constructed and in use today consist of two courses of material—a lower or base course and an upper course or wearing surface. The lower course usually consists of coarse crushed rock and a filler of graded aggregate and sand combined with a sufficient amount of bituminous binder to coat all the material. The upper course usually consists of fine crushed aggregate and sand, together with a bituminous binder, and in some instances of sand and a bituminous binder only. The two courses are spread hot and rolled and to all appearances when completed produce a pavement of considerable stability and with wear-resisting qualities. Numerous defects, however, usually develop in a pavement of this character in a comparatively short period of time. When the pavement is subjected to heavy traffic during hot weather, the wearing surface becomes soft and creeps, thereby producing a wavy or corrugated surface; the surface layer becomes thin in spots and soon wears through. The coarser rocks in the lower layer begin to shatter or abrade; water begins to penetrate and general disintegration takes place.

The object of the present invention is to generally improve and simplify the construction of pavements of the character described; to provide a wear-resisting surface which will not creep; to provide a pavement which is resilient and shock-absorbing in its upper portion; to provide a pavement with greater stability and compactness to resist displacement by traffic, and further to provide a method of laying the pavement whereby greater compactness is obtained and better unity and bond is secured between the several courses forming the pavement.

For convenience in describing the construction of the pavement forming the subject matter of the present invention, and the method of preparing and laying the same, reference will be made to the accompanying drawing which shows a vertical cross-section of a portion of the pavement. By reference to the drawing it will be noted that the pavement is laid in three courses—a bottom or lower course, "a", an intermediate course, "b", and a top course or wearing surface, "c". The upper course is composed chiefly of a fine mineral matter, rich in bituminous

binder to effectively resist abrasive action and suction from fast-moving, rubber-tired traffic. The intermediate layer forms a support for the above surface and is composed chiefly of a slightly coarser mineral matter containing a somewhat less quantity of bituminous binder. The intermediate layer also forms a covering for the lower layer and protects the coarser stones in the lower layer, and furthermore assists in producing stability throughout the entire pavement. The lower course is composed chiefly of coarse broken rock, or the like, and a filler consisting of a mixture of bituminous binder mixed with a graded, comparatively fine mineral matter. This course may be laid in any thickness from one inch to four inches. No coarse rock should, however, be employed which has a diameter that will equal more than three-fourths the thickness of the course. For instance, if the course is four inches thick, the coarse rock may be as large as three inches. The mineral aggregate which forms the filler between the coarse rock is graded so that a portion thereof consists of crushed rock or material which passes a one-half inch screen, another portion passing a one-fourth inch screen, another portion a ten-mesh screen, and still another portion will pass a 200-mesh screen. To this mineral aggregate is added from 2 to 7% by weight of bituminous binder. The aggregate and the binder, together with the coarse rock, is run through a dryer and a mixer where it is thoroughly heated and mixed with the binder, the aggregate, and the rock. The above mixture should be delivered to the roadway to be paved in a thoroughly heated condition and there dumped in the most convenient manner for handling. After dumping on the sub-grade indicated at "D", it is spread out with hot shovels or forks and when the required thickness is obtained it should be immediately rolled with a heavy roller, the rolling to be continued until the course has received about 75% of its final compression and while still hot it should be immediately covered with a second course mixture.

The second or intermediate course consists chiefly of a crushed rock or like material which passes a 1/2" screen. To this is added material passing a 1/4" screen, a 10-mesh screen and a 200-mesh screen. To this graded, comparatively fine aggregate is added from 4 to 8% by weight of bituminous

binder. The entire mixture is thoroughly heated, dried and mixed in the usual manner and should arrive ready for use at a temperature of from 250 to 500° F. It is then spread out to the required thickness and should be immediately subjected to a heavy roller. After rolling, if any low places are in evidence, an additional quantity of the mixture may be added to bring the surface to a true and even contour. After all low places have been filled in and thoroughly compressed and while still hot, the pavement is ready for the final surface course. This may consist of bituminous binder and sand alone, or it may consist of crushed material passing a 1/4" screen and mixed with finer material passing a 200-mesh screen, this graded aggregate being then mixed with 10 to 18% by weight of bituminous binder. This mixture is also heated and thoroughly mixed and is delivered to the pavement at a temperature ranging from 250 to 500° F. It is here spread to the required thickness and immediately rolled, the rolling being continued until no further compression may be obtained. In actual practice, where the total thickness of the pavement when completed is five inches, the upper course will not exceed one-fourth of an inch, the intermediate course will be approximately three-fourths of an inch, and the lower course four inches. All of the courses in this pavement can be produced by an ordinary paving plant designed to prepare hot mixed coarse aggregate pavements without additions or alterations. The mineral filler in all mixtures may be added cold, while the other ingredients are being mixed, if such method is more convenient providing the ingredients are sufficiently heated after the cold filler has been added. The bituminous binder used in this pavement should be soluble in cold carbon bisulphide, and it may be refined from tar, natural asphalt or petroleum oils. The penetration or hardness of the binder should be determined for each individual paving job after considering climatic conditions at the local point where the mixture is to be used for paving. The method of laying the pavement is also an important feature of the present application. In actual practise, it has been found that when the first course or layer of material is placed and rolled that chilling of the lower surface takes place due to contact with the sub-grade, and similarly that the upper surface chills rapidly due to contact with the roller. As a consequence, the entire body of material is not compressed to as high a compactness as might be desired, the center portion only of the course reaching a proper compactness as it retains its semi-plastic condition for the longest period of time. When the second or intermediate course is laid, it has a temperature

of from 250 to 500° F. The temperature is quickly conducted to the upper surface of the lower course and the surface is thus softened so that compactness is increased when the intermediate course is rolled. The heating of the upper surface of the lower course to increase its compactness when re-rolling is important, and re-heating is also important as it produces a closer unity or bond between the two layers. 75

The upper course when finally laid also has a high temperature of from 250 to 500° F., and as such reheats the upper portion of the intermediate layer. This is also important as the compactness thereof is increased when the upper course is rolled and a better bond is obtained between the intermediate and upper course. In fact, the entire compactness and stability of the pavement is materially increased by laying the several courses as described. 80

A pavement laid by this method is accordingly not only compact throughout but also contains great stability under traffic due to the bond formed by the layers and the interlocking effect obtained by the gradual grading of the aggregate with relation to the coarse rock in the lower layer. 90

The gradual grading of the mineral matter from coarse rock to fine is of further importance. For instance, when the first layer or lower course is laid and rolled a comparatively rough or uneven surface is obtained. If a wearing surface was placed directly thereon, it would be uneven in thickness and when subjected to heavy traffic in warm weather it would soon creep and become corduroyed. Not so in this instance. The rough surface obtained after rolling of the first course is covered by the intermediate layer and as this contains a comparatively fine aggregate or crushed rock, it may be raked and rolled to a substantially smooth surface or contour and as such presents an ideal surface for reception of the upper layer or wearing surface. This upper layer will accordingly be uniform in thickness and may be made exceedingly thin. As already stated, a quarter of an inch thickness is more than sufficient and may be laid even thinner if desired. This is a decided advantage, as experience has shown that a thin surface of uniform thickness has comparatively little, if any, tendency to creep. 105

By using the proportions of ingredients and by following the method described such as locating the different sizes of mineral aggregate in their proper places, a pavement is produced which is substantially monolithic in structure. The body of the pavement has great compactness and stability and two upper layers are formed which are not only wear-resisting and shock-absorbing, but which will also render the pavement impervious to moisture and disintegration. 120

When laying a pavement which is five inches thick, I prefer to use crushed rock and aggregates in substantially the following proportions:

5 In the lower course the crushed rock aggregates and fine material will conform to substantially the following grading: first—crushed rock not over 3" in size; retained upon a  $\frac{1}{2}$ " screen, 45 to 65%; passing a 10  $\frac{1}{2}$ " screen and retained upon a  $\frac{1}{4}$ " screen 8 to 20%; passing a  $\frac{1}{4}$ " screen and retained upon a 10-mesh screen, 8 to 15%; passing the 10-mesh screen, 8 to 28%. Of the material passing the 10-mesh screen, at least 15 8% should pass a 200-mesh screen. To this is added 2 to 7% by weight of bituminous binder.

20 The second course should comply to the following grading: crushed rock or like material retained upon a  $\frac{1}{2}$ " screen not to exceed 5%; passing the  $\frac{1}{2}$ " screen and retained upon a  $\frac{1}{4}$ " screen, 40 to 65%; passing the  $\frac{1}{4}$ " screen and retained upon a 10-mesh screen, 15 to 30%; passing the 10-mesh 25 screen and retained upon a 200-mesh screen, 8 to 25%, and passing the 200-mesh screen, 5 to 10%. To this is added 4 to 8% by weight of bituminous binder.

20 The surface course is composed of aggregate which should comply with the following grading: crushed rock or like material retained upon a  $\frac{1}{4}$ " mesh screen not to exceed 5%; passing the 10-mesh screen and retained upon a 200-mesh screen, 55 to 75%, and passing the 200-mesh screen, 15 to 30%. To this is added 10 to 18% by weight of bituminous binder.

When local material does not contain sufficient filler to conform to the above grading, 40 Portland cement, lime dust, carbonated lime, or other manufactured filler of approved quality, may be used to make up the shortage. In this specification, all material retained upon a 10-mesh screen is referred to 45 as crushed rock or stone. All material passing the 10-mesh screen and retained upon a 200-mesh screen is referred to as aggregate, and all material passing a 200-mesh screen

is referred to as fine aggregate or filling material.

Having thus described my invention, what I claim and desire to secure by Letters Patent is—

1. A method of constructing a bituminous pavement of the character described which comprises spreading a hot coarse aggregate bituminous concrete mixture in a layer approximately the thickness desired for the complete pavement, compressing it to approximately seventy-five percent of the compression it will take and while still hot covering it with a hot finer aggregate bituminous concrete mixture in a layer approximately one fourth the desired depth of the complete pavement, compressing it to approximately seventy-five percent of the compression it will take and while this mixture is still hot covering it with a still finer aggregate bituminous mixture and compressing the complete pavement into a single layer. 55

2. A bituminous pavement consisting of a single layer composed of three dissimilar bituminous mixtures so disposed that the lower three-fourths to four-fifths of the layer consists of a dense bituminous concrete composed principally of mineral particles three inches to one-half inch size; ninety-five percent of the upper one-fifth to one-fourth of the layer consisting of a finer aggregate bituminous concrete composed principally of 60 mineral particles one-half inch and one-fourth inch in size; and the uppermost five per cent of the layer consisting of a bituminous mixture in which all of the mineral particles are less than one-half inch and at 65 least ninety-five percent of them range from one-fourth inch size to filler which will pass a 200 mesh screen; the three mixtures being so combined during the process of laying and compressing that the result is a single 70 layer in the upper one-fourth of which the predominating size of the particles of mineral decreases to a minimum and the percentage of bituminous binder increases to a maximum at the top.

MORRIS L. GORDON.